

## UNITED STATES PATENT OFFICE.

WALTER O. SNELLING, OF ALLENTOWN, PENNSYLVANIA.

## CONCENTRATION OF TIN MINERALS

No Drawing.

Application filed October 31, 1925. Serial No. 66,105.

My invention relates to improvements in the treatment of ores of tin, and more particularly relates to an improved method of concentrating tin ores by superficial alteration of easily reducible tin minerals.

I have discovered that when a tin mineral such as cassiterite, the principal ore of tin, is subjected to reducing action, as by electrolytic reduction or the action of nascent 10 hydrogen, the surface of the mineral is partly or wholly reduced to metallic tin, and that the superficially reduced grains or particles may then be separated from other accompanying ore minerals or from gangue 15 material much more completely than by the methods of separation at present known.

As an example of my present invention I will describe the method which I may employ in the treatment of stream gravel containing cassiterite in association with quartz, calcite and like gangue minerals, as well as heavy minerals such as gold, galena and wolframite.

I first separate the lighter gangue minerals by means of tables or jigs, or any of the other customary milling operations, thus obtaining a concentrate, and I then pass this concentrate over amalgamated plates, to remove gold or other minerals that will be caught on the mercury surface. I then agitate the concentrate with lumps of zinc and dilute hydrochloric acid. After a short period of agitation the surface of all particles of cassiterite will assume a gray, metallic 30 appearance, due to the superficial reduction of the ore particles, and upon again running the concentrate over amalgamated plates, the cassiterite particles may be completely separated from other minerals that may be present, the superficial reduction of the surface of the tin mineral causing these particles to now adhere to the mercury on the plates.

The essential feature of my invention is the superficial reduction of particles of tin ore, and the utilization of the modified surface of the ore particles as a means of separating them from associated materials. Instead of employing amalgamated plates as the means of separation, I may employ flotation or any other suitable form of separation, the change in the surface of the tin ore as a result of reducing action being to so greatly modify the behavior of the ore particles as to make their separation from associated minerals very sharp and complete.

When employing flotation methods in the treatment of tin ores, I prefer to first subject the properly sized and graded mineral particles to selective flotation, and I then 60 treat the separated material containing the cassiterite by electrolytic reduction or by agitation in zinc drums containing dilute hydrochloric acid, or in wooden drums containing shot zinc and dilute hydrochloric 65 acid, until the surface of the cassiterite particles have been superficially reduced to metallic tin, after which I again subject the mineral mixture to flotation, by these steps obtaining a very sharp and complete separation. 70

The reason for the much more complete separation which I am able to obtain by the method herein outlined, as compared with any method of separation of tin minerals 75 which has ever been previously described, is to be found in the very wide difference in behavior towards separating operations which is offered by oxide surfaces and metal surfaces. In passing over an amalgamated plate, the oxide ores of tin show no tendency whatever to adhere to the plate, while after superficial reduction the ore particles show very great adhesion to the amalgamated 80 plate, and similarly in flotation the original cassiterite behaves as an oxide in the first flotation operation, and as a metal in the second flotation operation, thus again showing the maximum possible difference in separating 85 action. 90

The operation of superficial reduction of the cassiterite particles does not greatly change the specific gravity of the ore mineral, and very slight superficial action, such as may be obtained by electrolytic reduction 95 in from one to two minutes, or by the action of zinc and hydrochloric acid in from two to five minutes is sufficient to entirely change the behavior of the particles of tin ore toward an amalgamated plate or in a flotation 100 cell, and to enable the separation of the particles of tin ore to be made from other particles of heavy minerals that, by reason of similarity in specific gravity or in flotation characteristics, can not be separated or can only be separated with great difficulty by other common methods of separation now in use. 105

The ability to undergo superficial reduction with the formation of a surface film of 110 metal from the action of mild electrolytic reduction or from the action of nascent hy-

drogen or from the action of zinc and hydrochloric acid is practically specific to the mineral cassiterite, and accordingly the utilization of this remarkable and quite unique 5 characteristic of the mineral as a means of concentrating the "values" present in lean ore enables a remarkably clean and sharp separation to be made from other ore minerals.

10 Although my present invention has been described in connection with its use in the concentration of tin ores, it will of course be evident that the principle as herein described may be applied to the concentration of the 15 tin oxide dross from the metallurgical treatment of tin, or to the concentration of other fused or semi-fused tin oxide residues, or to tin oxide from any other source, preferably after being compressed, granulated, sintered 20 or fused, to make the material more amenable to physical handling and treatment.

It will be evident that many modifications 25 may be made without departing from the essential features of the disclosure as herein made, and accordingly no limitations should be imposed in connection with my invention except as indicated in the appended claims.

I claim:

1. In the treatment of minerals, the process 30 which comprises superficially reducing

particles of cassiterite electrolytically to metallic tin, and thereafter separating such superficially reduced particles from associated mineral particles.

2. In the treatment of tin ore the process 35 which comprises electrolytically reducing the surface of particles of a tin mineral partially to metallic tin, and thereafter utilizing the modified surface of such particles as a means of separation from other mineral 40 particles.

3. In the concentration of tin ore, the process which comprises subjecting the ore to a process of separation, electrolytically reducing the surface of tin minerals present 45 in the concentrate, and effecting a further concentration by retreating the concentrate by the process of separation previously employed.

4. In the concentration of tin ores, the process which comprises subjecting the ore to flotation treatment, reducing at least a portion of the surface of tin minerals in the concentrate to metallic tin, and again subjecting the concentrate to a further flotation 50 treatment.

In testimony whereof, I have hereunto subscribed my name this 30th day of October 1925.

WALTER O. SNELLING.